

## UNITED STATES PATENT OFFICE

2,614,929

## METHOD OF PREPARING PHOTOGRAPHIC EMULSIONS

Henry C. Yutzy and Frederick J. Russell, Rochester, N. Y., assignors to Eastman Kodak Company, Rochester, N. Y., a corporation of New Jersey

No Drawing. Application August 13, 1947,  
Serial No. 768,476

13 Claims. (Cl. 95—7)

1

This invention relates to a method for preparing washed silver-halide photographic emulsions in which the silver halide is prepared in a solution of gelatin, mixed with gelatin derivative, acid-coagulated, washed, and then re-dispersed.

Heretofore in the making of photographic emulsions gelatin has been principally depended upon as the carrier for the silver halide and as the peptizing agent employed in its preparation. In these normal methods of preparing silver-halide emulsions the emulsion maker has in the past been limited in the scope of his operations by the physical properties peculiar to gelatin. These characteristics have necessitated limitations on the concentration of silver halide and of gelatin in photographic emulsion formulae to values which are not most desirable for all purposes. For instance, emulsions of high concentration of silver halide have been difficult to prepare. Limitations have been imposed on the emulsion maker regarding the conditions of dilution during emulsion making since emulsions with too high water content are difficult and undesirable to coat. In addition, the technician has been obliged to limit the minimum concentration of gelatin in the washing operation in which soluble salts are removed. It has been the usual practice heretofore in preparing washed emulsions to set the dispersion of silver halide in gelatin to a jelly, noodle this jelly and wash by osmosis with cold water preferably with a hardener added thereto. Under such conditions a minimum gelatin concentration of approximately 3-4% is permissible, and this limitation has hampered the free operations of the emulsion maker in preparing emulsions of this type.

One object of our invention is to provide a method of preparing photographic emulsions of the washed type in which the difficulties previously met with are absent. Another object of our invention is to provide a method of washing silver-halide dispersions in which substantially all of the liquid may be removed therefrom in the course of the washing operation. A further object of our invention is to provide a method of preparing silver-halide dispersions using gelatin derivatives in their preparation. Other objects of our invention will appear herein.

We have found a ready means of avoiding the limitations which have heretofore been met with in the preparation of photographic emulsions. Our method is especially valuable in expanding the possible conditions for the manufacture of photographic silver-halide emulsions of different speeds, contrasts, and other photographic char-

2

acteristics. In addition, the method in accordance with our invention offers a simple means to prepare emulsions of high silver concentration which is especially valuable in the manufacture of films bearing large quantities of silver per unit area. In its broadest aspects, our invention involves the mixing of gelatin derivatives into dispersions of silver halide in gelatin in sufficient amount to impart coagulating properties to the entire mass. The gelatin derivatives which are employed in accordance with our invention may be prepared from gelatin by adjusting a solution or suspension of gelatin to a pH value of 8 to 11 or more with a suitable base, such as sodium hydroxide or ammonium hydroxide and then adding a reagent which will react therewith, ordinarily at a temperature of 25-60° C. The reaction between the reagent and the gelatin usually takes 5-20 minutes after which the gelatin derivative may be employed either in the solution in which it is formed or in solid condition. The gelatin derivatives which have been found to be especially useful in the process in accordance with our invention are those of the aromatic sulfonyl chlorides, the carboxylic acid chlorides, the carboxylic acid anhydrides, especially of the dicarboxylic type, the aryl isocyanates, and the 1,4-diketones. The following compounds have been found to be useful for preparing gelatin derivatives suitable for use in our invention:

## Sulfonyl chlorides

Benzene sulfonyl chloride  
35 p-Methoxybenzene sulfonyl chloride  
p-Phenoxybenzene sulfonyl chloride  
p-Bromobenzene sulfonyl chloride  
p-Toluene sulfonyl chloride  
m-Nitrobenzene sulfonyl chloride  
40 m-Sulfonylbenzoyl dichloride  
Naphthalene-beta-sulfonyl chloride  
p-Chlorobenzene sulfonyl chloride  
3-nitro-4-aminobenzene sulfonyl chloride  
m-Carboxy-4-bromobenzene sulfonyl chloride  
45 1-chlorosulfonyl-2-hydroxy-3-naphthoic acid  
quinoline-8-sulfonyl chloride  
m-Carboxybenzene sulfonyl chloride  
2-amino-5-methylbenzene-sulfonyl chloride

## Carboxylic acid chlorides

50 Phthalyl chloride  
p-Nitrobenzoyl chloride  
Benzoyl chloride  
Ethyl chlorocarbonate  
55 Furoyl chloride

## Acid anhydrides

Phthalic anhydride  
Benzoinic anhydride  
Succinic anhydride  
Maleic anhydride  
Isatoic anhydride

## Isocyanates

Phenyl isocyanate  
p-Bromophenyl isocyanate  
p-Chlorophenyl isocyanate  
p-Tolyl isocyanate  
p-Nitrophenyl isocyanate  
Alpha-naphthyl isocyanate  
Beta-naphthyl isocyanate

## 1,4-diketones

Acetonyl acetone  
Dimethyl acetonyl acetone

In its broadest aspects our invention comprises the formation of the silver-halide grains in an aqueous solution of gelatin whereby good dispersion is obtained followed by the addition to this solution of a gelatin derivative in sufficient proportion to impart coagulating properties to the entire mass. The amount of gelatin derivative which must be added to insure satisfactory coagulation is determined by two features: (1) the concentration of normal gelatin which is present and (2) the concentration of salt which is present in the solution. In the case of emulsions which contain alkali metal nitrate equivalent to the silver halide formed in the double decomposition reaction, the ratio of gelatin derivative to normal gelatin should be of the order of 4 to 1. If large quantities of salt are present, the ratio of the gelatin derivative to the gelatin may be as little as 2 to 1 for good emulsion coagulation properties.

In the process in accordance with our invention the silver-halide dispersion is prepared in normal gelatin in accordance with the usual procedure. The silver-halide formation and such ripening as is desired is carried out. There is then added to the silver-halide dispersion gelatin derivative in an amount which will give the mass the property of being acid coagulable. This may be a proportion of gelatin derivative of 2 to 1 derivative to gelatin, 4 to 1, or, if desired, an even larger proportion of gelatin derivative may be added, although as a practical matter, proportions of less than 10 to 1 are most satisfactory. The gelatin derivative is thoroughly stirred into the silver-halide dispersion whereupon acid is added to reduce the pH to less than 4.5, the amount of salt present determining the lower limit of the pH range. If the nitrate resulting as a by-product from the preparation of the silver halide is present, the pH may be reduced to 3 and coagulation will be obtained in this case, the salt being on the order of approximately 0.2 normal. If for some reason higher concentrations of salt are present, a still greater range of pH may be employed for the coagulation. Upon reducing the pH to the coagulation range, the gelatin derivative coagulates and carries down the gelatin and silver halide therewith. The phenomenon which occurs is characterized by an enveloping of the silver-halide grains by the coagulated gelatin derivative so that a grainy mass is obtained. This mass may then be subjected to repeated washings, thereby removing substantially all of the water-soluble salts from the coagulum.

For some types of emulsions the coagulum may 75

be employed directly without any further washing than the removal of the mother liquor from the precipitated material. For instance, in the preparation of emulsions for the coating of paper

5 and other permeable materials, extended washing is not necessary. However, in the preparation of emulsion for coating on film or glass, it is desirable to reduce the content of soluble salts below that which obtains in the coagulation after 10 the mother liquor has been removed therefrom. This washing may be done by any one of several methods. The coagulum may be rinsed by treatment with cool water, preferably with a pH adjusted to the isoelectric point of the gelatin derivative. The number of rinses necessary to reduce the salt content of the coagulum to the desired point is usually within the range of 1 to 4 changes of water. As an alternative method for washing the coagulum may be dissolved in water 15 at an elevated pH, such as by using water containing a small proportion of sodium or ammonium hydroxide to bring the pH of the mass up to 6 or more. The temperature of the mass is raised to approximately 40° C., and the whole 20 is stirred for a few minutes to effect re-dispersion of the coagulum. After complete re-dispersion has been obtained, the gelatin derivative may be coagulated by the addition of an appropriate acid solution to reduce the pH to the coagulation point 25 of the derivative. After the addition of the acid the coagulum will settle and is separated from the mother liquor in the same manner as in the first coagulation step. The coagulation and re-dispersion operation may be repeated as often as 30 necessary but for normal purposes one cycle of washing is sufficient.

35 The coagulum which has been washed by either of the two general methods outlined above may then be re-dispersed to form photographic emulsions suitable for the subsequent finishing and 40 coating operations by treating with the required quantity of water, normal gelatin or gelatin derivative and base to raise the pH of the whole to 5 or 6 or even greater. The mixture of coagulum, water, gelatin or gelatin derivative and any other materials which have been added is then 45 stirred at approximately 40° C. for the time required to effect complete re-dispersal of the coagulum. The time required is normally of the order of ten to twenty minutes but may vary 50 depending upon the chemical nature of the particular gelatin derivative used. The emulsion thus prepared behaves similarly to emulsions prepared using a similar emulsification and ripening technique in which noodle washing is employed. The emulsions prepared in accordance with our invention respond readily to the standard methods of chemical sensitization or after 55 ripening, and optical sensitization. They may be coated by the techniques usual in coating photographic emulsions. The use of gelatin derivatives for obtaining washed emulsions presents considerable advantage over other techniques described in the literature for the washing of emulsions. It has been well known for years that 60 gelatin silver-halide emulsions could be coagulated by the addition of sufficient quantities of suitable organic solvents of which methanol, ethanol, or acetone may serve as an example. Such 65 procedures, however, have proved to be expensive and cumbersome because of the very large quantities of organic solvent which must be used per unit of emulsion since no chemical reaction between the gelatin and the solvent is in question. The gelatin coagulates and becomes in-

soluble in the medium through the well-known effect of organic solvents to coagulate proteins.

In the preparation of gelatin-silver halide emulsions accompanied by the use of gelatin derivatives, the physical characteristics of water insolubility as related to pH are of vital importance. With gelatin derivatives water insolubility is exhibited within the pH range of approximately 4 to 4.5. In the presence of neutral electrolytes, however, the pH range of water insolubility is broadened and may extend from 3 to 4.5 or possibly even more. In the initial coagulation considerable neutral electrolyte is usually present in the form of potassium nitrate (or other alkali metal salts) resulting from the double decomposition reaction between silver nitrate and potassium bromide, for instance. In addition to this salt it is common practice that some soluble halide also be present. Under such conditions the adjustment of pH in the first coagulation is not particularly critical. If, however, the coagulum is re-dispersed, a second coagulation will take place at a much lower salt concentration and, therefore, the pH adjustment necessary will be more critical. For this purpose we prefer to operate in the range of 3.8 to 4.2.

It is apparent that considerable advantage will accrue by the use of this method in that the concentration of silver halide in the final emulsion may be adjusted to any desired value without reference to the quantities of water, silver halide, and gelatin used in the initial emulsification reaction. Therefore, emulsions may be prepared with very small water content. An additional advantage of the coagulum method of operation lies in the considerable reduction of equipment necessary, since the washing operation may be carried out in the usual emulsion-making equipment, and the additional operations and equipment necessary for the usual washing operation may be eliminated. We have found that the dicarboxylic acid anhydride derivatives of gelatin, such as of phthalic anhydride, are useful for preparing washed silver-halide dispersions and emulsions. These derivatives of gelatin and their preparation are described and claimed in Frame and Yutzy application, Serial No. 768,474, filed of even date, now Patent No. 2,525,753. We have found that the coagulation operation in accordance with our invention may be carried out either after the preparation of silver halide to remove water-soluble salts therefrom or after a heat treatment thereof with appropriate chemical sensitizers so that the coagulated silver-halide grains may be obtained either before or after having been brought to optimum photographic speed. These grains may be dried at either stage in the cycle without deleterious effect on their properties when finally made up in the emulsion. We have found that our invention may be carried out with any of the above-mentioned derivatives of gelatin without regard as to the gelatin which has been employed to form the derivative. Although we have found that the standard type of photographic gelatin is very satisfactory in preparing emulsions in accordance with our invention, we have also found that other types of gelatin, such as the hydrolyzed gelatins or glues having a lowered viscosity may be converted to gelatin derivatives and used in preparing washed emulsions in accordance with our process.

The following examples illustrate our invention:

Example 1.—100 g. of silver nitrate was dis-

solved in 900 cc. of distilled water at 25° C. In another vessel 80 g. of potassium bromide, 1 g. of potassium iodide and 25 g. of gelatin were dissolved in 900 cc. of distilled water. The temperatures of both solutions were adjusted to 50° C. and the silver nitrate solution was added to the potassium bromide-gelatin solution over a period of approximately ten minutes accompanied by vigorous stirring. During the addition of the silver nitrate solution and for ten minutes thereafter the temperature was maintained at 50° C. whereupon it was cooled to 40° C. One-half of this silver-halide dispersion was mixed with a solution of 75 g. of benzene sulfonyl chloride derivative of gelatin dissolved in 600 cc. of distilled water, thus rendering the dispersion acid coagulable. This gelatin derivative had been prepared by dissolving 100 g. of gelatin in 1100 cc. of distilled water, adjusting the pH to 9.5 with 20% sodium hydroxide and the temperature to 110° F. There was added to this solution 7 g. of benzene sulfonyl chloride over a period of ten minutes and the pH of 9.5 and the temperature of 110° F. were maintained during this addition and for 45 minutes thereafter. Dilute sulfuric acid was then added to lower the pH to 6 and the resultant mass of gelatin derivative was set, sliced, and dried.

After the gelatin derivative had been added to the silver-halide dispersion the dispersion was stirred for five minutes at 40° C., after which approximately 20 cc. of 5-N sulfuric acid were added to reduce the pH to 3.0. After standing at this pH for several minutes a coagulum of silver halide and gelatin settles out. The mother liquor was decanted off and the coagulum was redispersed in one liter of distilled water by stirring vigorously for five minutes at 40° C. There was then added to the emulsion approximately 15 cc. of 3 N ammonium hydroxide thereby raising the pH to 4.1 and causing recoagulation. After settling, the mother liquor was decanted off and the coagulum was redispersed in a gelatin solution containing 75 g. of gelatin and sufficient water to adjust the total weight to 1.36 kg. After stirring the mixture for twenty minutes at 40° C. to insure homogeneity, the emulsion was cooled to 30° C. and chilled in order to set it.

A 400 cc. portion of this emulsion was melted at 40° C. and 3 N ammonium hydroxide was added until the mixture was approximately neutral. A small amount of potassium bromide was added according to the procedure well known in the art, and the emulsion was subjected to a temperature of 65° C. until optimum speed, contrast, and reasonable fog were reached. For instance, the emulsion was coated on 5 x 7 glass plates, was chilled and dried and tested sensitometrically by exposure on a photographic sensitometer and development in a photographic developer.

Example 2.—To the second portion of the silver-halide dispersion prepared as described in the first paragraph of Example 1 there was added 75 g. of the phenyl isocyanate derivative of gelatin, thereby imparting to the dispersion the property of being acid coagulable. The gelatin derivative used here was prepared in the same manner as that of Example 1 except that phenyl isocyanate was employed instead of benzene sulfonyl chloride as the reagent. The coagulation, decantation, washing, and finishing of the emulsion followed the same procedure as in Example 1. An emulsion having good photographic properties was obtained.

Example 3.—The procedure of Example 1 was

followed except that 50 g. of a phthalic anhydride derivative of gelatin was used instead of the benzene sulfonyl chloride derivative. A dispersion was obtained which was acid coagulable. The gelatin derivative used here was prepared by adding 15 g. of phthalic anhydride in 100 cc. of dry acetone over a 23-minute period to a solution of 100 g. of gelatin in 1000 cc. of water, the mass being maintained at 40° C. and at a pH of 9.5. After ten minutes the pH was lowered to 7.0 with dilute sulfuric acid and the gelatin was chill set, sliced, washed, and dried. The coagulation, washing, and recoagulation were carried out in the same manner as described in the preceding examples. The finished emulsion prepared as described in Examples 1 and 2 was coated on glass plates and tested sensitometrically. This emulsion was found to have good photographic properties.

*Example 4.*—The same procedure was followed as in Example 1 except that 75 g. of m-carboxy benzene sulfonyl chloride derivative of gelatin was mixed with the silver-halide dispersion instead of the benzene sulfonyl chloride derivative. The derivative employed was prepared by adding 10.5 g. of m-carboxy benzene sulfonyl chloride in 50 cc. of dry acetone to a solution of 100 g. of gelatin in 900 cc. of water at 40° over a period of two hours. The pH of the gelatin solution was adjusted to 10.0 and maintained there by the use of 10% sodium hydroxide throughout the reaction. The pH was then adjusted to 7.0 with dilute sulfuric acid. The gelatin solution was set by chilling, sliced, washed and dried.

The emulsion obtained by the procedure described was washed by successive coagulations as described in Example 1, was brought to its final volume, and was finished and coated onto glass plates for sensitometric tests. A photographic emulsion having good properties was obtained.

*Example 5.*—The procedure described in Example 1 was followed except that in place of the benzene sulfonyl chloride derivative of gelatin 50 g. of p-tolyl isocyanate derivative of gelatin was mixed with the silver-halide dispersion and after reduction of the pH to produce a coagulum, the mother liquor was decanted therefrom and the coagulum was redispersed in distilled water at 40° C. Recoagulation was obtained by raising the pH to 4.1 with 3 N ammonium hydroxide. The mother liquor was decanted off and after redispersing the coagulum in 75 g. of gelatin and sufficient water to adjust the weight to 1.36 kg. the emulsion was finished in the same manner as in Example 1. A portion of the finished emulsion was coated on glass plates and sensitometric tests showed that it had good photographic properties.

*Example 6.*—The procedure of Example 1 was followed except that the derivative obtained by reacting maleic anhydride with gelatin was employed to impart acid coagulability to the silver-halide dispersion. The derivative employed was prepared by dissolving 50 g. of gelatin in 400 cc. of distilled water and adjusting the pH to 10 with 20% sodium hydroxide. The mass was then heated to 120° F. and 12.5 g. of maleic anhydride was added over a period of approximately three minutes, the pH being maintained close to 10 throughout the reaction which took approximately thirty minutes. The pH was lowered to 6 with dilute sulfuric acid, and the resulting solution was added directly to the silver-halide dispersion.

The coagulation, decantation, redispersion, re-

coagulation with ammonium hydroxide and final adjustment of the emulsion to its finishing volume and composition were carried out in the same manner as in Example 1. A portion of the finished emulsion was coated on glass plates and sensitometric tests showed that it had good photographic properties.

*Example 7.*—The same procedure was followed as described in Examples 1 and 6 except that a benzoyl chloride derivative of gelatin was used to confer acid coagulability on the silver-halide dispersion. This derivative was prepared by the same procedure as described in the preceding example except that in place of maleic anhydride 12.5 g. of benzoyl chloride was reacted with the gelatin solution. The emulsion obtained was coated on glass plates and upon testing sensitometrically was found to have good photographic properties.

*Example 8.*—The same procedure was followed as in Example 1 except that 75 g. of a furoyl chloride derivative of gelatin dissolved in 600 cc. of water was added to the emulsion in place of the benzene sulfonyl chloride derivative of gelatin to impart acid coagulability thereto. The method of preparing this derivative is described in U. S. application No. 768,472 of Gordon F. Frame, filed of even date, now Patent No. 2,494,041 issued January 10, 1950. The particular furoyl chloride derivative of gelatin used was prepared by reacting 100 parts of gelatin in 1200 parts of water at a pH of 10 at 104° F. with 7.5 parts of furoyl chloride in 50 parts of dry acetone. The pH was machined at 10 during the addition of the furoyl chloride and for fifteen minutes thereafter. The pH was then reduced to 6 with dilute sulfuric acid, and the mass was chilled, noddled, washed two hours, melted, chilled, sliced, and dried. The preparation of the emulsion and the washing procedure described in Example 1 were followed. After the emulsion was finished, it was coated onto glass plates, and sensitometric tests showed good photographic properties.

*Example 9.*—The procedure followed here was the same as that used in Example 7 except that the coagulum produced by acidifying the mixture of silver-halide dispersion and benzoyl chloride derivative of gelatin was washed twice in cold water before final dispersion in the gelatin solution. The ammonia coagulation described in Examples 7 and 1 was omitted. The final emulsion was finished by heat treatment and coated on glass plates as described in Example 7. Sensitometric tests showed that the emulsion had satisfactory photographic properties.

*Example 10.*—A silver-halide dispersion in gelatin was prepared as described in the first paragraph of Example 1. This dispersion was halved and to this half portion was added 50 g. of a benzoyl chloride derivative of gelatin as described in Example 7. To the resulting mixture 20 cc. of aqueous sulfuric acid was added to reduce the pH to 3. A coagulum of silver halide and gelatin formed and was allowed to settle. The mother liquor was decanted from the coagulum, and the latter was redispersed in one liter of distilled water at 40° C. and a pH of 6.5 obtained by adding approximately 15 cc. of 3 N ammonium hydroxide. The silver-halide dispersion was again coagulated by adding aqueous sulfuric acid to lower the pH of the mixture to 4.1, and the mother liquor was again decanted therefrom. The coagulum was dedispersed in a solution containing 75 g. of gelatin and sufficient

weight of water to bring the total weight to 1.36 kg. After stirring for twenty minutes at 40° C. the emulsion was finished by treating with heat and coating onto glass plates. The emulsion upon testing sensitometrically showed good photographic properties.

*Example 11.*—The procedure of the preceding example was followed except that the benzoyl chloride derivative of gelatin was prepared from a glue stock instead of from high viscosity gelatin. The procedure of coagulating, washing, and decanting, final adjustment of composition, and finishing described in the examples above gave an emulsion having good sensitometric properties.

*Example 12.*—The procedure described in Example 9 was followed except that the second half of the silver-halide dispersion prepared as described in Example 10 was employed with the exception that 75 g. of the benzoyl chloride derivative of glue (or unrefined gelatin) was employed to impart acid coagulating properties to the dispersion. The silver-halide dispersion was coagulated, decanted and washed in cold water. The coagulum was then dispersed in 75 g. of gelatin solution as the vehicle therefor and adjusted to a total weight of 1.36 kg. This mixture was stirred for twenty minutes at 40° C. and was then cooled to 30° C. and chilled. A test portion of 400 cc. was melted at 40° C. giving heat treatment for approximately forty minutes at 65° C. and was coated on glass plates. The plate coatings were exposed and were found to give good sensitometric results.

*Example 13.*—The following solutions were prepared: solution A, 200 cc. of aqueous solution containing 50% silver nitrate by weight; solution B, having a total volume of 200 cc. and containing 190 cc. of an aqueous solution containing 40% potassium bromide by weight and 9½ cc. of a solution containing 25% potassium iodide by weight, 65 g. of a polyvinyl alcohol solution containing 20.8% polyvinyl alcohol and 205 cc. of water stirred at 93° C. for fifteen minutes to assure complete solution of the polyvinyl alcohol. Then there was added 950 cc. of water, 100 cc. of 28% ammonium hydroxide and 20 g. of urea. There was then added at a temperature of 90° F. solutions A and B over a period of eleven minutes with good stirring. Solution B was added beginning fifteen seconds after beginning solution A. A small quantity of ethyl alcohol was added dropwise during this period to reduce foam. After the dispersion had been prepared 100 cc. of glacial acetic acid was added, and the mass was chilled to 20° C.

There was then added to the silver-halide dispersion 200 cc. of water containing 25 g. of a benzoyl chloride derivative of gelatin. This derivative was prepared by dissolving 50 g. of gelatin in 400 cc. of water, raising the pH to 10 with dilute aqueous sodium hydroxide and adding 12.5 g. of benzoyl chloride over a period of fifteen minutes with good stirring. The mass was maintained at a pH of 10 and a temperature of 40° C. for twenty-five minutes.

The pH of the mixture of the silver-halide dispersion and the gelatin derivative was reduced to 2 by the addition of aqueous sulfuric acid. The coagulum formed was allowed to settle, and the supernatant liquor was removed by decantation. The coagulum was washed twice in cold distilled water, the distilled water used for washing being adjusted to a pH of 3 with sulfuric acid. The washed coagulum was then redispersed in 500 cc. of distilled water by

adjusting the pH to 7.5 with dilute sodium hydroxide and stirring for twenty-five minutes at 50° C. The resulting emulsion was then cooled to 40° F., the pH was adjusted to 6 with dilute sulfuric acid and coated on standard photographic paper stock. Instead of polyvinyl alcohol or gelatin other peptizing colloids may be employed in the preparation of the silver-halide dispersions in accordance with our invention.

10 We claim:

1. In a method of preparing washed silver halide dispersions, the steps which comprise mixing a water-soluble silver salt and a water-soluble halide salt in an aqueous solution of a peptizing colloid, mixing therewith at least 2 parts of a gelatin derivative per part of the peptizing colloid, thereby rendering the silver halide dispersion coagulable at a pH within the range of pH 3-4.5, which gelatin derivative is selected from the group consisting of the aromatic sulfonyl chloride derivatives of gelatin, the carboxylic acid chloride derivatives of gelatin, the carboxylic acid anhydride derivatives of gelatin, the aromatic isocyanate derivatives of gelatin and the 1,4 diketone derivatives of gelatin, coagulating the dispersion of silver halide by adjusting to said pH whereby silver halide-peptizer-gelatin derivative grains are formed and subsequently separating those grains from the liquid portion of the mass.
2. In a method of preparing washed silver halide dispersions, the steps which comprise mixing a water-soluble silver salt and a water-soluble halide salt in an aqueous solution of gelatin as the peptizing colloid, mixing therewith at least 2 parts of a gelatin derivative per part of gelatin, thereby rendering the silver halide dispersion coagulable at a pH within the range of pH 3-4.5, which gelatin derivative is selected from the group consisting of the aromatic sulfonyl chloride derivatives of gelatin, the carboxylic acid chloride derivatives of gelatin, the carboxylic acid anhydride derivatives of gelatin, the aromatic isocyanate derivatives of gelatin and the 1,4 diketone derivatives of gelatin, coagulating the dispersion of silver halide by adjusting to said pH whereby silver halide-gelatin-gelatin derivative grains are formed and subsequently separating those grains from the liquid portion of the mass.
3. In a method of preparing washed silver halide dispersions, the steps which comprise mixing a water-soluble silver salt and a water-soluble halide salt in an aqueous solution of polyvinyl alcohol as the peptizing colloid, mixing therewith at least 2 parts of a gelatin derivative per part of polyvinyl alcohol, thereby rendering the silver halide dispersion coagulable at a pH within the range of pH 3-4.5, which gelatin derivative is selected from the group consisting of the aromatic sulfonyl chloride derivatives of gelatin, the carboxylic acid chloride derivatives of gelatin, the carboxylic acid anhydride derivatives of gelatin, the aromatic isocyanate derivatives of gelatin and the 1,4 diketone derivatives of gelatin, the carboxylic acid anhydride derivative by adjusting to said pH whereby silver halide-polyvinyl alcohol-gelatin derivative grains are formed and subsequently separating those grains from the liquid portion of the mass.
4. In a method of preparing washed silver halide dispersions, the steps which comprise mixing a water-soluble silver salt and a water-soluble halide salt in an aqueous solution of a peptizing colloid, mixing therewith at least 2 parts

of an aromatic sulfonyl chloride derivative of gelatin per part of the peptizing colloid, thereby rendering the silver halide dispersion coagulable at a pH within the range of pH 3-4.5, coagulating the silver halide dispersion by adjusting to said pH whereby silver halide-peptizer-gelatin derivative grains are formed and subsequently separating the thus-formed grains from the liquid portion of the mass.

5. In a method of preparing washed silver halide dispersions, the steps which comprise mixing a water-soluble silver salt and a water-soluble halide salt in an aqueous solution of a peptizing colloid, mixing therewith at least 2 parts of a carboxylic acid anhydride derivative of gelatin per part of the peptizing colloid, thereby rendering the silver halide dispersion coagulable at a pH within the range of pH 3-4.5, coagulating the silver halide dispersion by adjusting to said pH whereby silver halide-peptizer-gelatin derivative grains are formed and subsequently separating the thus-formed grains from the liquid portion of the mass.

6. In a method of preparing washed silver halide dispersions, the steps which comprise mixing a water-soluble silver salt and a water-soluble halide salt in an aqueous solution of gelatin as the peptizing colloid, mixing therewith at least 2 parts of a carboxylic acid anhydride derivative of gelatin per part of the peptizing colloid, thereby rendering the silver halide dispersion coagulable at a pH within the range of pH 3-4.5, coagulating the silver halide dispersion by adjusting to said pH whereby silver halide-peptizer-gelatin derivative grains are formed and subsequently separating the thus-formed grains from the liquid portion of the mass.

7. In a method of preparing washed silver halide dispersions, the steps which comprise mixing together a water-soluble silver salt and a water-soluble halide salt in an aqueous solution of a peptizing colloid, mixing therewith at least 2 parts of the benzene sulfonyl chloride derivative of gelatin per part of the peptizing colloid, thereby rendering the silver halide dispersion coagulable at a pH within the range of pH 3-4.5, coagulating the silver halide dispersion by adjusting to said pH whereby silver halide-peptizer-gelatin derivative grains are formed and subsequently separating those grains from the liquid portion of the mass.

8. In a method of preparing washed silver halide dispersions, the steps which comprise mixing together a water-soluble silver salt and a water-soluble halide salt in an aqueous solution of a peptizing colloid, mixing therewith at least 2 parts of the phenyl isocyanate derivative of gelatin per part of the peptizing colloid, thereby rendering the silver halide dispersion coagulable at a pH within the range of pH 3-4.5, coagulating the silver halide dispersion by adjusting to said pH whereby silver halide-peptizer-gelatin derivative grains are formed and subsequently separating those grains from the liquid portion of the mass.

9. In a method of preparing washed silver halide dispersions, the steps which comprise mixing together a water-soluble silver salt and a water-soluble halide salt in an aqueous solution of a peptizing colloid, mixing therewith at least 2 parts of the phthalic anhydride derivative of gelatin per part of the peptizing colloid, thereby rendering the silver halide dispersion coagulable at a pH within the range of pH 3-4.5, coagulating the silver halide dispersion by adjusting to

said pH whereby silver halide-peptizer-gelatin derivative grains are formed and subsequently separating those grains from the liquid portion of the mass.

5. 10. In a method of preparing washed silver halide dispersions, the steps which comprise mixing together a water-soluble silver salt and a water-soluble halide salt in an aqueous solution of a peptizing colloid, mixing therewith at least

10 2 parts of the benzoyl chloride derivative of gelatin per part of the peptizing colloid, thereby rendering the silver halide dispersion coagulable at a pH within the range of pH 3-4.5, coagulating the silver halide dispersion by adjusting to

15 said pH whereby silver halide-peptizer-gelatin derivative grains are formed and subsequently separating those grains from the liquid portion of the mass.

11. In a method of preparing washed silver halide dispersions, the steps which comprise mixing water-soluble silver salt and water-soluble halide salt in an aqueous solution of gelatin as the peptizing colloid, mixing therewith at least 2 parts of the phthalic anhydride derivative

25 of gelatin per part of the peptizing colloid, thereby rendering the silver halide dispersion coagulable at a pH within the range of pH 3-4.5, coagulating the silver halide dispersion by adjusting to said pH whereby silver halide-peptizer-

30 gelatin derivative grains are formed and subsequently separating those grains from the liquid portion of the mass.

12. A method of preparing a washed silver halide photosensitive emulsion which comprises mixing a water-soluble silver salt and a water-soluble halide salt in an aqueous solution of a peptizing colloid, mixing therewith at least 2

35 parts of the phthalic anhydride derivative of gelatin per part of the peptizing colloid, thereby rendering the silver halide dispersion coagulable at a pH within the range of pH 3-4.5, coagulating the silver halide dispersion by adjusting to

40 said pH whereby silver halide-peptizer-gelatin derivative grains are formed, separating those grains from the liquid portion of the mass and subsequent by mixing those grains with gelatin and water as a protective colloid for the silver halide whereby a photosensitive emulsion is formed.

50 13. In a method of preparing washed silver halide dispersions, the steps which comprise mixing a water-soluble silver salt and a water-soluble halide salt in an aqueous solution of a peptizing colloid, mixing therewith approximately

55 4 parts of a gelatin derivative per part of the peptizing colloid, thereby rendering the silver halide dispersion coagulable at a pH within the range of pH 3-4.5, which gelatin derivative is selected from the group consisting of the aromatic sulfonyl chloride derivatives of gelatin, the carboxylic acid chloride derivatives of gelatin,

60 the carboxylic acid anhydride derivatives of gelatin, the aromatic isocyanate derivatives of gelatin and the 1,4 diketone derivatives of gelatin, coagulating the dispersion of silver halide by

65 adjusting to said pH whereby silver halide-peptizer-gelatin derivative grains are formed and subsequently separating those grains from the liquid portion of the mass.

70

HENRY C. YUTZY.

FREDERICK J. RUSSELL.

13

## REFERENCES CITED

The following references are of record in the  
file of this patent:

## UNITED STATES PATENTS

| Number    | Name            | Date          |
|-----------|-----------------|---------------|
| 1,844,716 | Lambert         | Feb. 9, 1932  |
| 2,139,774 | Sheppard et al. | Dec. 13, 1938 |
| 2,282,001 | Russell et al.  | May 5, 1942   |

Number  
2,489,341

14

Name  
Waller

Date  
Nov. 29, 1949

## FOREIGN PATENTS

| 5 Number | Country       | Date           |
|----------|---------------|----------------|
| 479,419  | Great Britain | Feb. 4, 1938   |
| 537,256  | Great Britain | June 16, 1941  |
| 580,504  | Great Britain | Sept. 10, 1946 |